

Aug. 8, 1972

KEIZO SANO ET AL  
POLYESTER FILAMENTS HAVING AN IMPROVED  
WATER-ABSORBING PROPERTY

3,682,846

Filed Oct. 27, 1969

4 Sheets-Sheet 1

FIG.1



FIG.2



FIG.3



FIG.4



Aug. 8, 1972

KEIZO SANO ET AL  
POLYESTER FILAMENTS HAVING AN IMPROVED  
WATER-ABSORBING PROPERTY

Filed Oct. 27, 1969

3,682,846

4 Sheets-Sheet 2

FIG.5



FIG.6



FIG.7



FIG.8



Aug. 8, 1972

KEIZO SANO ET AL  
POLYESTER FILAMENTS HAVING AN IMPROVED  
WATER-ABSORBING PROPERTY

3,682,846

Filed Oct. 27, 1969

4 Sheets-Sheet 3

FIG.9



FIG.10



FIG.11



FIG.12



Aug. 8, 1972

KEIZO SANO ET AL  
POLYESTER FILAMENTS HAVING AN IMPROVED  
WATER-ABSORBING PROPERTY

3,682,846

Filed Oct. 27, 1969

4 Sheets-Sheet 4



Fig. 13



Fig. 14

**1**

3,682,846

**POLYESTER FILAMENTS HAVING AN IMPROVED WATER-ABSORBING PROPERTY**

Keizo Sano, Nagaizumi-machi, Taigi Watanabe, Mishimashi, Michihiko Tanaka, Nagaizumi-machi, Yoshimitsu Ichikawa, Mishima-shi, Koichi Kato, Otsu-shi, and Hirokichi Matsuura, Mishima-shi, Japan, assignors to Toray Industries, Inc., Tokyo, Japan

Filed Oct. 27, 1969, Ser. No. 869,731

Int. Cl. C08j 1/14, 1/28

U.S. Cl. 260—2.5 N

9 Claims

**ABSTRACT OF THE DISCLOSURE**

Polyester filaments containing therein 0.4—5% by weight of a polyalkylene ether and 0.3—3% by weight of a metal salt derivative, and having fine pores aligned in the direction of the filament axis.

This invention relates to polyester filaments having an improved water-absorbing property which is not degraded by repetition of washing. More specifically, it relates to polyester filaments containing 0.4 to 5% by weight of a polyalkylene ether and 0.3 to 3% by weight of a metal salt derivative and having fine pores aligned in the direction of the filament axis.

The conventional techniques for imparting a water-absorbing property to polyester filaments will be described below.

(A) Attempts to render polyester filaments hydrophilic by copolymerizing a polyester with a polyether compound have been proposed in Japanese patent application publications Nos. 10,336/61, 4,312/64 and 15,095/63, British Patent No. 682,866 specification, and U.S. Patent No. 2,744,087 specification.

However, in accordance with methods proposed in these references it is difficult to impart a sufficient water-absorbing property to polyester filaments without deterioration of their thermal and mechanical properties.

(B) Methods comprising blending a polyether in the dispersed state into a polyester have been known from Japanese patent application publications Nos. 5,214/64 and 14,613/66. However, in accordance with these known methods it is impossible to impart a sufficient water-absorbing property to polyester filaments without deterioration of their thermal and mechanical properties.

(C) A method comprising blending a ring-containing vinyl polymer in a polyester and eluting the blended polymer to thereby form fine pores in the polyester has been known from Japanese patent application publication No. 4,815/66.

However, this method fails to impart a water-absorbing property to polyesters.

(D) In view of the description of Example 2 of the specification of Japanese patent application publication No. 5,214/64 it is presumed that there was obtained a fibrous composition of a polyester containing a polyethylene glycol and having fine pores. In accordance with the teachings of this reference it is possible to impart to polyester filaments a temporary water-absorbing property but the said water-absorbing property is abruptly degraded by repetition of washing. Therefore, the filaments obtained in accordance with the teachings of this reference are of little utility.

(E) A method comprising making a polyalkylene ether and an alkali metal sulfonate derivative present in a polyester has been known from Italian Patent No. 796,237 specification. However, in accordance with this method it is impossible to impart a water-absorbing property to polyester filaments.

**2**

As results of our researches made with a view to overcoming defects of these prior arts, particularly shortcomings that a sufficient water-absorbing property cannot be imparted to polyester filaments, an attempt to impart a sufficient water-absorbing property to polyester filaments results in deterioration of their thermal and mechanical properties, and that if a water-absorption property is once imparted to polyester filaments, said property is not sufficiently resistant to washing, we arrived at the present invention. Accordingly, a primary object of this invention is to impart to polyester filaments an everlasting and sufficient water-absorbing property without deterioration of their thermal and mechanical properties.

This object of the present invention can be attained by polyester filaments containing 0.4—5% by weight of a polyalkylene ether and 0.3—3% by weight of a metal salt derivative and having fine pores aligned in the direction of the filaments axis.

The "polyester" referred to in this invention is a polyester in which at least 60% of the recurring units is composed of polyethylene terephthalate. For instance, it includes polyethylene terephthalate; copolymers obtained by copolymerizing polyethylene terephthalate with a known dicarboxylic acid component, dihydroxy component or hydroxycarboxylic acid component; polyester blends obtained by melt mixing an ethylene terephthalate homopolymer or copolymer with other homopolyester or copolyester; copolymers comprising an ethylene terephthalate homopolymer or copolymer and containing therein amide, urethane, ether, carbonate or other linkages; a fiber-forming polyester other than polyethylene terephthalate; and a fiber-forming polyester ether.

Of course, the above cited polymers may contain known catalysts, coloration inhibitors, heat stabilizers, antistatic agents, optical whitening agents, antiflaming agents, dyes, pigments and inactive fine particles.

The "polyalkylene ether" referred to in this invention is a polymer whose main chain is composed chiefly of alkylene ether units. For instance, it includes polyethylene oxide, polypropylene oxide, an ethylene oxide-propylene oxide copolymer, a mixture of polyethylene oxide and polypropylene oxide, a polymer derived from tetrahydrofuran, and a polymer derived from 1,3-dioxane. These polymers may have a group —OH, —OR or —O—CO—R (in which R is a monovalent organic group which may be optionally substituted) as the terminal group. Two or more of these terminal groups may be present in the polymer. In addition, a polymer blocked with phosphoric acid or a phosphate may be advantageously used. However, it is not preferable to use a modified polyalkylene ether which is made completely inactive by converting all the terminal groups to —OR groups.

It is preferable that the polyalkylene ether has a number average molecular weight exceeding 4,000. The use of a polyalkylene ether having too low a molecular weight is not preferred because a blend of the polyester and such a low molecular weight polyalkylene ether is inferior in spinnability and drawability.

Of course, the polyalkylene ether may contain known oxidants, catalysts and other additives.

The blending of the polyalkylene ether into the polyester may be performed by any method. For instance, it is possible to add a polyalkylene ether to a polymerization vessel for polyester at the time of initiation of the polymerization, during the polymerization or after completion of the polymerization. It is also possible to blend a polyalkylene ether with the use of an extruder into a polyester pelletized after completion of the polymerization. Further, it is possible to mix a solid polyester with a polyalkylene ether by means of a blender and then melt spin the mixture. Still further, it is possible to melt a poly-

ester and a polyalkylene ether separately and mix the melts by means of a screw just prior to the spinning. In order to attain the object of the present invention it is most preferable to add a polyalkylene ether to a polymerization vessel for the preparation of a polyester after completion of the polymerization, or to melt a polyalkylene ether and a polyester separately and mix the melts with the use of a screw just prior to the spinning.

The "metal salt derivative" referred to in this invention includes derivatives of alkali metal sulfonates, derivatives of metal salts of carboxylic, phosphonic and sulfonic acids, and derivatives of di- or mono-metal salts of phosphoric and phosphorous acids.

These metal salts will be detailed hereinbelow.

The "alkali metal sulfonate derivative" referred to in this invention includes compounds having a so-called surface-activating property, more specifically compounds having a hydrophobic group other than the sulfonic group. It is especially preferable to use a compound having only one sulfonic group at one end of its molecule.

Typical instances of such derivative are sodium dodecylbenzenesulfonate, potassium dodecylbenzenesulfonate, sodium nonylbenzenesulfonate and sodium 3-nonylphenoxypyropanesulfonate. But, the derivative is not limited to these specifically mentioned salts. It is not preferred to use an alkali metal sulfonate derivative having two or more sulfonic groups in the molecule, because such compound is not well blended with a polyester and resulting filaments are likely to have poor properties.

The "metal salt derivative of a carboxylic, phosphonic or sulfonic acid" includes surface-activating compounds containing in the molecule at least one hydrophobic group (which corresponds to the metal salt portion of an acid such as carboxylic acid) and a suitable hydrophobic group such as an alkyl group.

As such salt derivative there are cited following compounds but it is not limited to these specifically exemplified compounds:

- (1)  $C_8H_{17}COONa$
- (2)  $C_8H_{27}COOK$
- (3)  $C_{18}H_{37}COONa$
- (4)  $C_{12}H_{25}-O-CH_2COONa$
- (5) 
$$\begin{array}{c} O \\ || \\ C_{12}H_{25}-P-ONa \\ | \\ ONa \end{array}$$
- (6) 
$$\begin{array}{c} O \\ || \\ C_9H_{19}-\text{C}_6\text{H}_4-\text{C}_6\text{H}_4-P-ONa \\ | \\ ONa \end{array}$$
- (7) 
$$\begin{array}{c} O \\ || \\ C_9H_{19}-\text{C}_6\text{H}_4-\text{C}_6\text{H}_4-P-O-Mn \\ | \\ O-Mn \end{array}$$
- (8) 
$$\begin{array}{c} O \\ || \\ C_{12}H_{25}-\text{C}_6\text{H}_4-P-OK \\ | \\ OK \end{array}$$
- (9) 
$$\begin{array}{c} C_8H_{17}COO \\ | \\ C_8H_{17}COO \\ | \\ Zn \\ | \\ C_8H_{17}COO \end{array}$$
- (10) 
$$\begin{array}{c} C_9H_{19}-\text{C}_6\text{H}_4-O-\text{C}_6\text{H}_4-C_9H_{19} \\ | \\ NaO-P-ONa NaO-P-ONa \\ | \\ O \\ | \\ O \end{array}$$
- (11) 
$$\begin{array}{c} C_{12}H_{25}-S-O-ONa \\ | \\ O \end{array}$$



5 These metal salt derivatives should not possess an ester-linkage-forming group. In case a metal salt derivative containing an ester-linkage-forming group is used, the water-absorbing property of the resulting polyester filaments is very low, and it tends to impose bad influences on properties of the polyester filaments.

10 So-called surface-activating compounds having in the molecule at least one hydrophilic group (corresponding to the metal salt portion of an acid) and a hydrophobic group such as an alkyl group are preferably used in the present invention as the di- or mono-metal salt of phosphoric or phosphorous acid.

15 Such compounds are used in the form of a mono- or di-metal salt, and those in which the remaining  $-OH$  groups of phosphoric or phosphorous acid are converted to alkylaryl ester forms are preferably used. Further, it is preferable to use compounds which are free of ester-linkage-forming groups such as an acid group or hydroxyl group other than the phosphoric acid ester portion. The 20 reason is that such ester-linkage-forming group reacts with a polyester when the mono- or di-metal salt derivative of phosphoric or phosphorous acid is blended into the polyester, resulting in occurrence of an undesirable modification of the polyester.

25 Compounds having the following structures may be applied to this invention, but the mono- or di-metal salt derivative of the phosphoric or phosphorous acid is not limited to these specifically mentioned examples in the present invention.

- 30 (1) 
$$\begin{array}{c} ONa \\ | \\ C_{12}H_{25}-O-P-ONa \\ | \\ ONa \end{array}$$
- (2) 
$$\begin{array}{c} C_{12}H_{25}-O \\ | \\ C_{12}H_{25}-O-P-OK \\ | \\ C_{12}H_{25}-O \end{array}$$
- (3) 
$$\begin{array}{c} C_9H_{19}-\text{C}_6\text{H}_4-O-P-ONa \\ | \\ ONa \end{array}$$
- (4) 
$$\begin{array}{c} C_9H_{19}-\text{C}_6\text{H}_4-O-P-O-Mn \\ | \\ O \end{array}$$
- 35 (5) 
$$\begin{array}{c} C_9H_{19}-\text{C}_6\text{H}_4-O-P-ONa \\ | \\ O \\ | \\ ONa \end{array}$$
- (6) 
$$\begin{array}{c} C_9H_{19}-\text{C}_6\text{H}_4-O-P-O-Mn \\ | \\ O \\ | \\ O \end{array}$$
- 40 (7) 
$$\begin{array}{c} C_{12}H_{25}-O \\ | \\ C_{12}H_{25}-O-P-ONa \\ | \\ O \end{array}$$
- (8) 
$$\begin{array}{c} C_{12}H_{25}-O-P-OK \\ | \\ O \\ | \\ OK \end{array}$$
- 45 (9) 
$$\begin{array}{c} C_9H_{19}-\text{C}_6\text{H}_4-(OCH_2CH_2)_3O-P-ONa \\ | \\ O \end{array}$$
- 50 (6) 
$$\begin{array}{c} C_9H_{19}-\text{C}_6\text{H}_4-O-P-O-Mn \\ | \\ O \\ | \\ O \end{array}$$
- (7) 
$$\begin{array}{c} C_{12}H_{25}-O \\ | \\ C_{12}H_{25}-O-P-ONa \\ | \\ O \end{array}$$
- 55 (8) 
$$\begin{array}{c} C_{12}H_{25}-O-P-OK \\ | \\ O \\ | \\ OK \end{array}$$
- (9) 
$$\begin{array}{c} C_9H_{19}-\text{C}_6\text{H}_4-(OCH_2CH_2)_3O-P-ONa \\ | \\ O \end{array}$$
- 60 (7) 
$$\begin{array}{c} C_9H_{19}-\text{C}_6\text{H}_4-O-P-O-Mn \\ | \\ O \\ | \\ O \end{array}$$
- (8) 
$$\begin{array}{c} C_{12}H_{25}-O-P-ONa \\ | \\ O \\ | \\ ONa \end{array}$$
- 65 (9) 
$$\begin{array}{c} C_{12}H_{25}-O-P-OK \\ | \\ O \\ | \\ OK \end{array}$$
- 70 (10) 
$$\begin{array}{c} C_9H_{19}-\text{C}_6\text{H}_4-(OCH_2CH_2)_3O-P-ONa \\ | \\ O \end{array}$$

The blending of the above mentioned metal salt derivative may be performed by any method. It is possible to blend the metal salt derivative into the polyester either together with a polyalkylene ether or separately. The 75

blending may be carried out before the initiation of the polymerization for the preparation of a polyester, during the polymerization, or after completion of the polymerization. The salt derivative may be added to a polymerization vessel or blended by means of an extruder or blender. It is also possible to conduct the blending of the metal salt derivative just prior to the spinning. In the case of a mono- or di-metal salt derivative of phosphoric or phosphorous acid, it is preferable to blend it into the polyester after completion of the polymerization.

The present invention will be detailed by referring to drawings.

FIG. 1 is a microscopic photo illustrating the side of filaments from a blend obtained by incorporating polyethylene glycol into polyethylene terephthalate containing sodium dodecylbenzenesulfonate. The figure illustrates the stage that the polyethylene glycol is aligned in the polyethylene terephthalate along the filament axis. Since the filaments have not fine pores, they take a transparent appearance. FIG. 2 is a microscopic photo illustrating the side of filaments of this invention. As they have fine pores aligned along the filament axis, they possess a non-transparent appearance.

FIG. 3 is an electromicroscopic photo of the filaments of FIG. 1 after they have been dyed with osmium tetroxide ( $OsO_4$ ) and then dissolved. It is observed that the osmium tetroxide is adsorbed in the polyether portion and that the polyether component is blended in the state extended in the direction of the filament axis.

FIG. 4 is an electromicroscopic photo of filaments of the present invention prepared by eluting the polyether portion from the filaments of FIG. 1, after they have been dyed with osmium tetroxide and then dissolved. In this figure the stripe looks thinner because of the existence of fine interior pores than in FIG. 3.

FIG. 5 is a microscopic photo illustrating the side of polyester filaments from a blend obtained by incorporating polyethylene glycol into polyethylene terephthalate containing a di-sodium salt of nonylbenzenephosphonic acid. FIG. 6 is a microscopic photo illustrating the side of polyester filaments according to this invention.

FIG. 7 is an electromicroscopic photo of polyester filaments of FIG. 5, after they have been dyed with osmium tetroxide and then dissolved. FIG. 8 is an electromicroscopic photo of polyester filaments of the present invention obtained by eluting the polyether portion from polyester filaments shown in FIG. 5, after they have been dyed with osmium tetroxide and then dissolved.

FIG. 9 is a microscopic photo illustrating the side of polyester filaments incorporated with a di-sodium salt of nonylphenolphosphoric acid ester. FIG. 10 is a microscopic photo illustrating the side of polyester filaments of the present invention.

FIG. 11 is an electromicroscopic photo of filaments shown in FIG. 9, after they have been dyed with osmium tetroxide and then dissolved. FIG. 12 is an electromicroscopic photo of polyester filaments of the present invention obtained by eluting the polyether portion from polyester filaments shown in FIG. 9, after they have been dyed with osmium tetroxide and then dissolved.

The "fine pores aligned in the direction of the filament axis" referred to in the present invention indicate pores being present in the filament and having a diameter of  $0.01\mu$  to  $3\mu$  and a length-to-diameter ratio of at least 5.

As shown in FIGS. 2, 4, 6, 8, 10 and 12, the presence of fine pores is confirmed by observation under an optical microscope or electromicroscope. It is preferable that the ratio of the pore volume to the filament volume is within a range from 0.5 to 10%. In case the pore volume ratio is too small, the intended object of the present invention cannot be attained. On the other hand, in case the pore volume ratio is too great, the mechanical properties of the filaments are lowered.

The formation of fine pores may be performed by any method. For instance, it is possible to adopt a method

comprising treating filaments with warm water or a dilute aqueous alkali solution to thereby elute a blended polyalkylene ether. By such treatment the amount of the polyalkylene ether blended into polyester filaments is decreased, and pores such as shown in FIGS. 2, 4, 6, 8, 10 and 12 are formed in the filaments. In case the amount of the polyalkylene ether is not decreased even by such treatment, the existence of pores such as shown in FIGS. 2, 4, 6, 8, 10 and 12 is not observed.

It is also possible to adopt a method blending into a polyester a polymer incompatible with the polyester such as polyamide and polyolefin in addition to a polyalkylene ether and a metal salt derivative and eluting the blended polymer from the blend with a solvent for said blended polymer.

It is most preferable to adopt a method comprising eluting a part of a blended polyalkylene ether with a dilute aqueous alkali solution, while leaving the remaining part of the polyalkylene ether in the filament-constituting material.

During the formation of fine pores a part of the metal salt derivative is necessary stripped off from the filaments.

The amount of the polyalkylene ether finally contained in the filaments is within a range from 0.4 to 5% by weight, preferably from 1 to 4% by weight.

In case the amount of the polyalkylene ether is too small, the intended object of the present invention cannot be attained. On the other hand, in case the amount of the polyalkylene ether is too large, thermal and mechanical properties of the filaments are lowered.

The amount of the metal salt derivative finally contained in the filaments is within a range from 0.3 to 3% by weight, preferably from 0.3 to 2.5% by weight.

In case the amount of the metal salt derivative is too small, the intended object of the present invention cannot be attained. In case the amount of the metal salt derivative is too large, the mechanical properties of the filaments are degraded.

According to this invention there are provided polyester filaments having an excellent water-absorbing property and its excellent retainability. Reasons why such excellent effects are attained in accordance with the present invention have not been completely elucidated. Only blending of a polyalkylene ether and a metal salt derivative into filaments does not result in manifestation of any water-absorbing property. The synergistic action of fine pores and the polyalkylene ether and metal salt derivative contained in filaments produces the abovementioned effects.

Further, the filaments of this invention retain excellent physical properties inherent to polyester fibers and possess an excellent antistatic property at the same time.

This invention will be now detailed by referring to examples.

In examples the "parts" indicate "parts by weight." The analysis of the polyalkylene ether component was conducted in accordance with the method of Robert (Robert, J. Levins and Robert, M. Ikeda, *Analy. Chem.* 37, 671 (1965)) after decomposing the polymers with aminopropanol and neutralizing the same with acetic acid.

The analysis of the alkali metal sulfonate derivative was conducted by a method comprising depolymerizing the polymers with ethylene glycol, forming an aqueous solution of the depolymerized polymers, making the solution acidic with sulfuric acid, adding methylene blue thereto, extracting the resulting complex and subjecting it to colorimetric determination.

The amount incorporated of the derivative of a metal salt of a carboxylic, phosphonic or sulfonic acid was determined by the analysis of the metal content according to the atomic absorptiometric method.

The amount incorporated of the di- or mono-metal salt of phosphoric or phosphorous acid was determined by the analysis of the metal content according to the atomic absorptiometric method.

The inherent viscosity of the polymer was measured in o-chlorophenol at 25° C.

The evaluation of physical properties of filaments was based on CR values of wooly-processed yarns. CR values are values indicating the crimp retainability of the processed yarns. Higher values mean that yarns are more excellent in the crimp retainability and the bulkiness. The measurement of CR values is conducted in the following manner:

The sample is subjected to a boiling water treatment under a load of zero for 5 minutes. Then, the sample is taken out from boiling water, thrown into water and allowed to stand therein for 1 minute under a load of 0.1 g./d. The length ( $L_1$ ) of the sample was measured. Then, the sample was taken out from water and allowed to stand under a load of 0.02 g./d. for 30 seconds. The length ( $L_2$ ) of the sample was measured again. The CR value of the sample was calculated by the following equation:

$$\text{CR Value} = \frac{L_1 - L_2}{L_1} \times 100$$

The heat resistance was evaluated based on changes in color of the sample when it was allowed to stand still in a hot air drier maintained at 180° C. for 5 hours.

The coloration was evaluated based on  $b$  values measured by employing a Hunter-type color machine of Japan Color Machine Co. (a high positive  $b$  value means an increase in coloration in yellow).

The evaluation of the water-absorbing property was conducted in the following manner:

The sample was allowed to stand at 20° C. and a relative humidity of 65% for 24 hours. Then, three sheets of the sample were piled up. Thereafter, 30  $\mu$ l. of water was dropped onto the piled sheets and the period of time from the initiation of the dropping to the point when any reflecting light from the surface of water having expanded on the sample was not observed (the time being called "water absorption time") was measured. A smaller value of the water absorption time means a higher water-absorbing property of the sample.

The washing treatment was conducted in the following manner:

15 liters of water at 40° C. was filled in a washing machine of an automatic reverser type of Toshiba Electric Co. and 26 g. of an anionic, weakly alkaline soap ("Zab" of Kao Soap Co.) was added thereto. The washing was carried out for 15 minutes and the washed sample was rinsed for 15 minutes in flowing clean water.

FIG. 13 illustrates an apparatus in use for another evaluation of filaments. More specifically, the apparatus is used for evaluation of the water-absorbing property of knitted products. In FIG. 13, the numerical reference 1 indicates a fine tube containing water therein, and the reference numeral 2 designates a water pool connected with the fine tube 1. The numeral reference 3 indicates

The oozing water is absorbed in the sample 4 and then released into the air through the sample 4. In case the sample has an excellent water-absorbing property, the amount of water passing through the fine tube 1, water pool 2, unglazed plate 3 and sample 4 should be great. Therefore, the amount consumed of water was read from the scale on the fine tube 1, and based on the read value the water-absorbing property was evaluated. In FIG. 13, the reference numeral 6 represents a water supply tank.

FIG. 14 is a graph illustrating the results of the actual measurements made on several samples by employing the apparatus of FIG. 13. In FIG. 14, the ordinate denotes the amount consumed (cc.) of water and the abscission represents the time (minutes).

#### 15 EXAMPLE 1 AND COMPARATIVE EXAMPLE 1

Polyethylene terephthalate (A) of an intrinsic viscosity of 0.660 obtained by a customary method was weighed at 295° C. by a gear pump and then fed to a 20 kneading screw portion heated at 285° C. A 2:1 mixture (B) of polyethylene glycol having a number average molecular weight of 20,000 and sodium dodecylbenzenesulfonate was weighed at 85° C. by a gear pump and fed to the kneading screw portion heated at 285° C.

25 The mixing ratio of (A):(B) was 92.5:7.5. The mixture was transferred from the kneading screw portion to a spinneret portion while being kept in the molten state. Then, the mixture was spun at a rate of 30 g./min. through a spinneret having 36 holes of a diameter of a 30 0.23 mm. and taken up at a rate of 1000 m./min. to obtain undrawn filaments. Then, the undrawn filaments were drawn at a draw ratio of 3.66 at a speed of 400 m./min. by means of a hot pin maintained at 100° C.

35 The resulting drawn filaments were characterized by a fineness of 75.1 d., a strength of 4.8 g./d., an elongation of 27.2% and a boiling water shrinkage of 11.5%.

Two of the so obtained filaments were gathered together and subjected to a wooly-processing at a yarn feed rate of 49.8 m./min., and a take-up rate of 44.0 m./min. with the use of a spindle rotating at 175,000 r.p.m. and a hot plate maintained at 205° C. Thus, there was obtained a wooly-processed yarn having a strength of 4.3 g./d., an elongation of 31.5% and a CR value (crimp retaining property) of 35.6%.

40 A knitted cloth of a weight of  $15-18 \times 10^{-3}$  gm./cm.<sup>2</sup> was formed from the so obtained wooly-processed yarn. Then, the knitted cloth was scoured at 80° C. for 20 minutes under the conditions of a cleanser of 2 g./liter, soda ash of 1 g./liter and a bath ratio of 1:100. Further, the knitted cloth was treated with a 0.3 N aqueous solution of sodium hydroxide at a bath ratio of 1:100 for 20 minutes at the boiling point of the solution. Before and after the above alkali treatment, the weight decrease ratio, and the amounts of polyethylene glycol and sodium dodecylbenzenesulfonate in the knitted cloth were measured. The results are shown in Table 1 below.

TABLE 1

|                                                    | Weight decrease ratio, percent | Amount of polyethylene glycol, percent | Amount of sodium dodecylbenzenesulfonate, percent |
|----------------------------------------------------|--------------------------------|----------------------------------------|---------------------------------------------------|
| Comparative Example 1 (before alkali treatment)... | 0                              | 4.9                                    | 2.5                                               |
| Example 1 (after alkali treatment).....            | 8.5                            | 1.8                                    | 1.1                                               |

an unglazed plate adhering closely to water, and the reference numeral 4 represents a knitted product sample on which a perforated plate 5 formed of polymethyl methacrylate is placed so as to regulate the form of the sample. Air is blown to the sample with an angle of 45° with respect to the sample surface at a rate of 0.5 m./sec. by means of an air blaster 6. The atmosphere is maintained at 20° C. and a relative humidity of 65%. The water in the fine tube 1 and the water pool 2 rises and oozes out on the surface of the unglazed plate 3 in such a manner as if the sweat comes out from the human body.

65 Optical microscopic photos illustrating the sides of the drawn yarn before the scouring and alkali treatments and of the drawn yarn after said treatments are shown in FIGS. 1 and 2. FIG. 3 is an electromicroscopic photo of the yarn of FIG. 1 after it has been dyed with osmium tetroxide and then dissolved. FIG. 4 is an electromicroscopic photo of the yarn of FIG. 2 after it has been dyed with osmium tetroxide and then dissolved. From the results shown in Table 1, and FIGS. 1 to 4 it is seen that in the yarn before the alkaline treatment the polyethylene glycol was incorporated in the form of stripes

and that a part of the polyethylene glycol corresponding to 3.1% of the total yarn was stripped off by the alkali treatment to form fine pores. It is also seen that in addition to the polyethylene glycol and sodium dodecylbenzenesulfonate, the polyethylene terephthalate per se was stripped off in an amount of 4.0% by the alkali treatment and hence, the yarn was made thinner and the pores were expanded from their interiors. From FIG. 4 it is also seen that the diameter of the pore was about  $0.1\mu$  and the length-to-diameter ratio was greater than 10.

With respect to the knitted cloth of the yarn before the alkali treatment and the knitted cloth of the yarn after the alkali treatment, the water-absorbing property was measured. The results are shown in Table 2 below.

TABLE 2

|                                                      | Before washing          | After 10 washings       | After 50 washings     |
|------------------------------------------------------|-------------------------|-------------------------|-----------------------|
| Comparative Example 1 (before alkali treatment)..... | More than 10 minutes.   | More than 10 minutes... | More than 10 minutes. |
| Example 1 (after alkali treatment).....              | Less than one second... | Less than one second... | Less than one second. |

From the results shown in Table 2 it is seen that even filaments containing polyethylene glycol and sodium

5 These examples are given to show what phenomena are brought about by changing the amounts incorporated of polyethylene glycol and sodium dodecylbenzenesulfonate in the polyester of Example 1.

10 The experiments were conducted in the same manner as in Example 1 except changing the mixing ratio of polyethylene glycol and sodium dodecylbenzenesulfonate, the incorporation ratio of the mixture of polyethylene glycol and sodium dodecylbenzenesulfonate to polyethylene terephthalate, or the amounts of polyethylene glycol and

sodium dodecylbenzenesulfonate incorporated into the polyester. The results are shown in Table 5 below.

TABLE 5

|                                                                        | Comparative Example 2 | Comparative Example 3 | Example 2           | Comparative Example 4 | Comparative Example 5 |
|------------------------------------------------------------------------|-----------------------|-----------------------|---------------------|-----------------------|-----------------------|
| Amount incorporated of polyethylene glycol (percent).....              | 5.0                   | 15.0                  | 5.0                 | 5.0                   | 1.0                   |
| Amount incorporated of sodium dodecylbenzenesulfonate (percent).....   | 0                     | 0                     | 5.0                 | 10.0                  | 1.0                   |
| Properties of woolly-processed yarn:                                   |                       |                       |                     |                       |                       |
| Strength (g./d.).....                                                  | 4.5                   | 3.9                   | 4.4                 | 3.8                   | 4.6                   |
| Elongation (percent).....                                              | 30.6                  | 28.1                  | 31.2                | 27.2                  | 32.0                  |
| CR value (percent).....                                                | 31.6                  | 20.3                  | 30.6                | 18.5                  | 31.8                  |
| After alkali treatment:                                                |                       |                       |                     |                       |                       |
| Weight decrease ratio (percent).....                                   | 7.1                   | 16.3                  | 10.2                | 10.3                  | 6.1                   |
| Amount of polyethylene glycol (percent).....                           | 2.1                   | 5.5                   | 1.9                 | 1.7                   | 1.0                   |
| Amount of sodium dodecylbenzenesulfonate (percent).....                | 0                     | 0                     | 2.1                 | 4.2                   | 1.0                   |
| Water-absorbing property:                                              |                       |                       |                     |                       |                       |
| Before washing.....                                                    | Less than 1 second.   | Less than 1 second.   | Less than 1 second. | Less than 1 second.   | 2 seconds.            |
| 10 washings.....                                                       | 1 second              | 1 second              | do                  | do                    | More than 10 minutes. |
| 50 washings.....                                                       | 5 minutes             | 4 minutes             | 1 second            | do                    | do                    |
| Heat resistance after alkali treatment (change in <i>b</i> value)..... | +1.9                  | +3.6                  | +2.1                | +7.7                  | +1.8                  |

dodecylbenzenesulfonate cannot possess a water-absorbing property unless they have fine pores therein.

Table 3 shows the results of the measurement of the heat resistance of the knitted cloths of the yarn before the alkali treatment and of the yarn after the alkali treatment.

TABLE 3

| Example No.:                                         | Heat resistance<br>(change in <i>b</i> value) |
|------------------------------------------------------|-----------------------------------------------|
| Comparative Example 1 (before alkali treatment)..... | +2.0                                          |
| Example 1 (after alkali treatment).....              | +1.8                                          |

For comparison sake, properties of ordinary polyester filaments (control) prepared without addition of polyethylene glycol and sodium dodecylbenzenesulfonate were examined. The spinning, drawing, woolly-processing, knitting and alkali treatment were conducted in the same manner as described above. The drawn yarn was characterized by a fineness of 74.9 d., a strength of 4.7 g./d., and elongation of 27.3% and a boiling water shrinkage of 11.3%. The woolly-processed yarn was characterized by a strength of 4.5 g./d., an elongation of 33.4% and a CR value of 35.6%, and the weight decrease ratio by the alkali treatment was 2.3%. The water-absorbing property of the knitted cloth was as follows:

TABLE 4

|                              | Before washing          | After 10 washings       | After 50 washings     |
|------------------------------|-------------------------|-------------------------|-----------------------|
| Before alkali treatment..... | More than 10 minutes... | More than 10 minutes... | More than 10 minutes. |
| After alkali treatment.....  | 5 minutes               | do                      | do                    |

The heat resistance expressed in terms of the change in *b* value of the knitted was +1.5 either before or after the alkali treatment.

From the results shown in Table 5 the following matters can be seen.

As in the case of Comparative Example 2, the filaments 45 containing polyethylene glycol and having pores therein but being free of sodium dodecylbenzenesulfonate are inferior in washing resistance of the water-absorbing property. As in the case of Comparative Example 3, even if the amount of polyethylene glycol is increased in Comparative 50 Example 2, the washing resistance of the water-absorbing property is not improved, and moreover the heat resistance and the CR value of the processed yarn are lowered. As in the case of Comparative Example 4, in case the amount of sodium dodecylbenzenesulfonate is too large, the CR 55 value of the processed yarn is low and the heat resistance is degraded. As in Comparative Example 5, even if filaments contain polyethylene glycol and sodium dodecylbenzenesulfonate and the weight decrease is observed after 60 the alkali treatment, a sufficient water-absorbing property is not imparted to the filaments when the weight decrease is due only to the surface falling and the polyethylene glycol contained in the form of stripes inside the filaments is not extracted. Thus, it is seen that the results given in 65 Table 5 demonstrate clearly the effects of the present invention.

#### COMPARATIVE EXAMPLE 6

This example is given to show that a sufficient water-75 absorbing property is not given to filaments containing only

an alkali metal sulfonate derivative, filaments obtained by subjecting the above filaments to an alkaline treatment and filaments containing an alkali metal sulfonate derivative and having fine pores therein.

To polyethylene terephthalate of Example 1, 2.5% of sodium dodecylbenzenesulfonate was added after completion of the polymerization. Thus, there was obtained a polymer having an intrinsic viscosity of 0.655.

The so obtained polymer (A) was weighed at 295°C. by means of a gear pump and fed to a kneading screw portion heated at 285°C. Polystyrene (B) ("Styron 666", product of Asahi Dow Chemical Industry Co.) was weighed at 180°C. by means of a gear pump and fed to the kneading screw portion heated at 285°C. The mixing ratio of (A) to (B) was 90:10.

Thereafter, the spinning, drawing, processing and knitting were conducted in the same manner as in Example 1, and then the polystyrene was eluted with trichlene at its boiling point. The weight decrease ratio was 9.1% at this treatment. It was confirmed that the filaments after the elution treatment contained sodium dodecylbenzenesulfonate in an amount of 1.0%. Thus, it is seen that the polystyrene portion incompatible with the polyester had been eluted out from the filaments and there were contained fine pores in the filaments. The water-absorbing property of the so treated filaments was characterized by 3 minutes before washing, more than 10 minutes after 10

Prior to the initiation of the preparation of polyethylene terephthalate, polyethylene glycol having a molecular weight of 20,000 was added to the polymerization system in an amount of 3.1% by weight based on the resulting polymer, and 2.5% by weight of sodium dodecylbenzenesulfonate was added after completion of the polymerization. Thus, there was obtained a polymer having an intrinsic viscosity of 0.663. In the same manner as in Comparative Example 6, the polymer was blend-spun with polystyrene, drawn, processed, knitted and treated with trichlene. After the trichlene treatment the amount incorporated of polyethylene glycol was 3.0%, and the amount incorporated of sodium dodecylbenzenesulfonate was 1.0%. The polystyrene in an amount of 9.0% was eluted out and fine pores were formed.

The water-absorbing property of the product was characterized by 1.0 second after 50 washings.

#### EXAMPLES 4 TO 7 AND COMPARATIVE EXAMPLES 7 TO 8

These examples are given to show what changes are brought about when the class of the polyalkylene ether to be incorporated is varied.

The experiments were conducted in the same manner as in Example 1 except changing the class of the polyalkylene ether to be incorporated. The results of the experiments are shown in Table 6 below.

TABLE 6

|                                                                    | Example 4                          | Comparative Example 7             | Example 5                         | Example 6                                                | Comparative Example 8             | Example 7                         |
|--------------------------------------------------------------------|------------------------------------|-----------------------------------|-----------------------------------|----------------------------------------------------------|-----------------------------------|-----------------------------------|
| Class of polyalkylene.                                             | Polypropylene glycol. <sup>1</sup> | Polyethylene glycol. <sup>2</sup> | Polyethylene glycol. <sup>1</sup> | Ethylene oxide/pro-pylene oxide co-polymer. <sup>3</sup> | Polyethylene glycol. <sup>4</sup> | Polyethylene glycol. <sup>5</sup> |
| Properties of processed yarn:                                      |                                    |                                   |                                   |                                                          |                                   |                                   |
| Strength (g./d.)                                                   | 4.6                                | 4.0                               | 4.3                               | 4.6                                                      | 4.3                               | 4.4                               |
| Elongation (percent)                                               | 30.1                               | 28.7                              | 30.0                              | 32.2                                                     | 30.1                              | 29.8                              |
| CR value (percent)                                                 | 29.8                               | 21.3                              | 25.2                              | 31.0                                                     | 28.6                              | 29.3                              |
| After alkali treatment:                                            |                                    |                                   |                                   |                                                          |                                   |                                   |
| Weight decrease ratio (percent)                                    | 7.8                                | 7.7                               | 8.0                               | 8.0                                                      | 8.0                               | 7.8                               |
| Amount incorporated of polyalkylene ether (percent)                | 1.0                                | 4.8                               | 2.3                               | 1.1                                                      | 0.2                               | 1.6                               |
| Amount incorporated of sodium dodecylbenzenesulfonate (percent)    | 1.2                                | 1.1                               | 1.0                               | 1.3                                                      | 1.3                               | 1.2                               |
| Water-absorbing property:                                          |                                    |                                   |                                   |                                                          |                                   |                                   |
| Before washing                                                     | Less than a second.                | 2 minutes                         | Less than 1 second.               | Less than 1 second.                                      | 5 seconds                         | Less than 1 second.               |
| After 10 washings                                                  | do                                 | More than 10 minutes.             | 7 seconds                         | do                                                       | More than 10 minutes.             | do                                |
| After 50 washings                                                  | 1 second                           | do                                | do                                | do                                                       | do                                | 5 seconds.                        |
| Heat resistance after alkali treatment (change in $\delta$ value). | +2.5                               | +3.0                              | +2.5                              | +2.0                                                     | +2.0                              | +1.9                              |

<sup>1</sup> Having a molecular weight of 6,000.

<sup>2</sup> Having a molecular weight of 600.

<sup>3</sup> Having a molecular weight of 21,000 (copolymerization ratio = 1:1).

<sup>4</sup> Both terminal ends of which are blocked with  $-\text{OCH}_3$  (molecular weight = 16,000).

<sup>5</sup> One terminal end of which is blocked with phosphoric acid (molecular weight = 10,000).

washings and more than 10 minutes after 50 washings. The water-absorbing property of a knitted product of the filaments prepared without addition of polystyrene by conducting the spinning, drawing, processing and knitting in the same manner as above was characterized by more than 10 minutes before washing. The water-absorbing property of a knitted product obtained by subjecting the above mentioned knitted product to an alkali treatment with a weight decrease ratio of 6.1% was characterized by 3 minutes before washing and more than 10 minutes after 10 washings. In this alkali-treated knitted product the content of sodium dodecylbenzenesulfonate was 1.0%, and fine pores were not formed in the filaments because sodium dodecylbenzenesulfonate was compatible with the polyester.

#### EXAMPLE 3

This example is given to show that even when fine pores are formed by a method different from the method adopted in Example 1, the effects of the present invention can be fully achieved.

From the results shown in Table 6 the following matters can be seen:

In Comparative Example 7, since the polyethylene glycol was not selectively eluted and fine pores were not formed, the filaments did not exhibit a sufficient water-absorbing property. In comparative Example 8, since the content of the polyalkylene ether in the filaments was too small, the filaments did not exhibit a sufficient water-absorbing property. Thus, it is seen that the results given in Table 6 demonstrate clearly the effects attained by the present invention.

#### EXAMPLES 8 AND 9

These examples are given to show what changes are brought about by varying the class of the alkali metal sulfonate derivative in Example 1.

The experiments were conducted in the same manner as in Example 1 except using other alkali metal sulfonate derivatives instead of sodium dodecylbenzenesulfonate.

The results are shown in Table 7 below.

TABLE 7

|                                                                    | Example 8                     | Example 9                         |
|--------------------------------------------------------------------|-------------------------------|-----------------------------------|
| Class of alkali metal sulfonate derivative                         | Sodium nonyl-benzenesulfonate | Potassium dodecylbenzenesulfonate |
| Properties of processed yarn:                                      |                               |                                   |
| Strength (g/d.)                                                    | 4.2                           | 4.1                               |
| Elongation (percent)                                               | 34.2                          | 33.6                              |
| CR value (percent)                                                 | 36.0                          | 34.8                              |
| After alkali treatment:                                            |                               |                                   |
| Weight decrease ratio (percent)                                    | 8.3                           | 8.5                               |
| Amount incorporated of polyethylene glycol (percent)               | 1.6                           | 1.3                               |
| Amount incorporated of alkali metal sulfonate derivative (percent) | 1.0                           | 0.9                               |
| Water-absorbing property:                                          |                               |                                   |
| Before washing                                                     | Less than 1 second            | Less than 1 second                |
| 10 washings                                                        | do                            | Do                                |
| 50 washings                                                        | do                            | 1 second                          |
| Heat resistance (change in <i>b</i> value)                         | +2.0                          | +2.3                              |

#### EXAMPLES 10 TO 11 AND COMPARATIVE EXAMPLES 9 TO 10

These examples are given to show what changes are brought about by varying the mixing method of polyethylene glycol (X) and sodium dodecylbenzenesulfonate (Y) in Example 1.

#### EXAMPLES 12 TO 13 AND COMPARATIVE EXAMPLES 11 TO 15

Frictional electrification voltages of various knitted products were measured at 20° C. and a relative humidity of 43% by means of a rotary static tester. The results are shown in Table 9.

TABLE 9

| Sample                 | Frictional electrification voltage (v.) |
|------------------------|-----------------------------------------|
| Example 12             | 2,300                                   |
| Comparative Example 11 | 9,800                                   |
| Comparative Example 12 | 7,000                                   |
| Comparative Example 13 | 6,500                                   |
| Example 13             | 2,100                                   |
| Comparative Example 14 | 8,100                                   |
| Comparative Example 15 | 7,200                                   |

In these examples the amounts mixed of (X) and (Y) are the same as in Example 1. The drawn yarns were of 40 75 deniers and 36 filaments. The spinning and drawing conditions were made as equal to those of Example 1 as possible. The processing, knitting and alkali treatment conditions were quite the same as those adopted in 45 Example 1.

The results are shown in Table 8 below.

It is seen that the results given in Table 9 clearly demonstrate the effects attained by the present invention.

#### EXAMPLE 14 AND COMPARATIVE EXAMPLES 16 TO 18

These examples are given to show the correspondence of the water-absorption time used as the criterion for evaluation of the water-absorbing property to the stuffy uncomfortable feeling of wearers.

TABLE 8

|                                                                 | Example 10                                                                                       | Example 11                                                                | Comparative Example 9                                                             | Comparative Example 10                                                                                                  |
|-----------------------------------------------------------------|--------------------------------------------------------------------------------------------------|---------------------------------------------------------------------------|-----------------------------------------------------------------------------------|-------------------------------------------------------------------------------------------------------------------------|
| Mixing method                                                   | (Y) was added to the polymerization vessel and mixed with (X) by extruder, followed by spinning. | (X) and (Y) were added to the polymerization vessel after polymerization. | (X) was added to the polymerization vessel, and (Y) was incorporated by extruder. | (X) was added to the polymerization vessel before polymerization, and (Y) was added to the vessel after polymerization. |
| Properties of processed yarn:                                   |                                                                                                  |                                                                           |                                                                                   |                                                                                                                         |
| Strength (g/d.)                                                 | 4.4                                                                                              | 4.3                                                                       | 4.4                                                                               | 4.2                                                                                                                     |
| Elongation (percent)                                            | 31.6                                                                                             | 32.3                                                                      | 31.6                                                                              | 32.6                                                                                                                    |
| CR value (percent)                                              | 34.3                                                                                             | 35.6                                                                      | 32.6                                                                              | 36.2                                                                                                                    |
| After alkali treatment:                                         |                                                                                                  |                                                                           |                                                                                   |                                                                                                                         |
| Weight decrease ratio (percent)                                 | 8.8                                                                                              | 8.2                                                                       | 7.3                                                                               | 6.9                                                                                                                     |
| Amount incorporated of polyethylene glycol (percent)            | 1.7                                                                                              | 1.5                                                                       | 4.8                                                                               | 4.9                                                                                                                     |
| Amount incorporated of sodium dodecylbenzenesulfonate (percent) | 1.2                                                                                              | 1.3                                                                       | 1.1                                                                               | 1.3                                                                                                                     |
| Water-absorbing property:                                       |                                                                                                  |                                                                           |                                                                                   |                                                                                                                         |
| Before washing                                                  | Less than 1 second                                                                               | Less than 1 second                                                        | 3 minutes                                                                         | 4 minutes                                                                                                               |
| 10 washings                                                     | do                                                                                               | 1 second                                                                  | More than 10 minutes                                                              | More than 10 minutes                                                                                                    |
| 50 washings                                                     | 1 second                                                                                         | 10 seconds                                                                | do                                                                                | Do                                                                                                                      |
| Heat resistance (change in <i>b</i> value)                      | +1.7                                                                                             | +1.9                                                                      | +2.3                                                                              | +2.6                                                                                                                    |

In comparative examples, since (X) was copolymerized with the polyester and hence (X) was not selectively eluted at the alkali treatment, fine pores were not formed and filaments having a water-absorbing property could not be obtained.

With respect to each of a knit underwear of the product of Example 1, a knit underwear of the control product described in Example 1, a knit underwear of Comparative Example 2, and a commercially available knit under-

wear of pure cotton having a weight of  $17 \times 10^{-3}$  g./cm.<sup>2</sup>, 10 men having an age of 20 to 25 years put on such knit underwear and were allowed to stay for 3 hours at a room maintained constantly at 27° C. and a relative humidity

treatment, the weight decrease, the amount of polyethylene glycol and the amount of disodium nonylbenzenephosphonate were measured. The results are shown in Table 11 below.

TABLE 11

|                                                  | Weight decrease ratio, percent | Amount of polyethylene glycol, percent | Amount of disodium nonylbenzenephosphonate, percent |
|--------------------------------------------------|--------------------------------|----------------------------------------|-----------------------------------------------------|
| Comparative Example 19 (before alkali treatment) | 0                              | 5.0                                    | 2.4                                                 |
| Example 15 (after alkali treatment)              | 8.2                            | 1.9                                    | 1.0                                                 |

of 65%, and the number of men complaining of a stuffy uncomfortable feeling was recorded. The tests were conducted with respect to either the underwears before washing or the underwears after 50 washings. The results are shown in Table 10.

TABLE 10

| Sample                 | Number of men complaining of stuffy uncomfortable feeling |                   |
|------------------------|-----------------------------------------------------------|-------------------|
|                        | Before washing                                            | After 50 washings |
| Example 14             | Underwear of the product of Example 1                     | 1                 |
| Comparative Example 16 | Underwear of the control product described in Example 1   | 9                 |
| Comparative Example 17 | Underwear of the product of Comparative Example 2         | 2                 |
| Comparative Example 18 | Underwear of pure cotton                                  | 1                 |

#### EXAMPLE 15 AND COMPARATIVE EXAMPLE 19

Polyethylene terephthalate (A) of an intrinsic viscosity of 0.660 containing 0.5% of titanium oxide as a delustering agent and obtained by a customary method was weighed at 295° C. by means of a gear pump, and then fed to a kneading screw portion heated at 285° C. A 2:1 mixture (B) of polyethylene glycol having a number average molecular weight of 20,000 and disodium nonylbenzenephosphonate was weighed at 85° C. by means of a gear pump and fed to the kneading screw portion heated at 285° C.

The mixing ratio of (A) and (B) was 92.5:7.5. The mixture was transferred from the kneading screw portion to a spinneret portion while being kept in the molten state. Then, the molten mixture was spun at a rate of 30 g./min. through a spinneret having 36 nozzles of a 0.23 mm. diameter. The extrudate was taken up at a rate of 1000 m./min. to obtain undrawn filaments. Thereafter, the filaments were drawn at a draw ratio of 3.66 at a

15 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905

acterized by a fineness of 73.8 d., strength of 4.9 g./d., an elongation of 26.4% and a boiling water shrinkage of 11.5%. The wooly-processed yarn was characterized by a strength of 4.5 g./d., an elongation of 32.8% and a CR value of 36.3%. The weight decrease ratio by the alkali treatment was 2.2%. The water-absorbing property of the knitted cloth was as follows:

TABLE 14

|                              | Before washing        | After 10 washings     | After 50 washings     |
|------------------------------|-----------------------|-----------------------|-----------------------|
| Before alkali treatment..... | More than 10 minutes. | More than 10 minutes. | More than 10 minutes. |
| After alkali treatment.....  | 5 minutes.....        | do.....               | Do.                   |

The heat resistance expressed in terms of the change in *b* value of the knitted cloth was +1.5 either before or after the alkali treatment.

#### EXAMPLES 16 AND COMPARATIVE EXAMPLES 20 TO 23

These examples are given to show what phenomena are brought about by changing the amounts incorporated of polyethylene glycol and disodium nonylbenzenephosphonate in the polyester of Example 15.

The experiments were conducted in the same manner as described in Example 15 except changing the mixing ratio of polyethylene glycol and disodium nonylbenzenephosphonate, the incorporation ratio of the mixture of polyethylene glycol and disodium nonylbenzenephosphonate to polyethylene terephthalate, or the amounts of polyethylene glycol and disodium nonylbenzenephosphonate incorporated in the polyester. The results are shown in Table 15 below.

This example is given to show that a sufficient water-absorbing property is not imparted to filaments containing only disodium nonylbenzenephosphonate, filaments obtained by subjecting the above filaments to an alkali treat-

ment, and filaments containing disodium nonylbenzenephosphonate and having fine pores therein.

To polyethylene terephthalate of Example 15, 2.5% of disodium nonylbenzenephosphonate was added after completion of the polymerization. Thus, there was obtained a polymer having an intrinsic viscosity of 0.657.

The so obtained polymer (A) was weighed at 295°C. by means of a gear pump and fed to a kneading screw portion heated at 285°C. Polystyrene (B) ("Styron 666", product of Asahi Dow Chemical Industry Co.) was weighed at 180°C. by means of a gear pump and fed to the kneading screw portion heated at 285°C. The mixing ratio of (A) to (B) was 90:10.

Thereafter, the spinning, drawing, processing and knitting were conducted in the same manner as in Example 15, and then the polystyrene was eluted with trichlene at its boiling point. The weight decrease ratio was 9.0% at this elution treatment. It was confirmed that the fila-

TABLE 15

|                                                                        | Comparative Example 20  | Comparative Example 21  | Example 16              | Comparative Example 22  | Comparative Example 23    |
|------------------------------------------------------------------------|-------------------------|-------------------------|-------------------------|-------------------------|---------------------------|
| Amount incorporated of polyethylene glycol (percent).....              | 5.0.....                | 15.0.....               | 5.0.....                | 5.0.....                | 1.0.....                  |
| Amount incorporated of disodium nonylbenzenephosphonate (percent)..... | 0.....                  | 0.....                  | 5.0.....                | 10.0.....               | 1.0.....                  |
| Properties of wooly-processed yarn:                                    |                         |                         |                         |                         |                           |
| Strength (g./d.).....                                                  | 4.4.....                | 4.0.....                | 4.3.....                | 3.7.....                | 4.5.....                  |
| Elongation (percent).....                                              | 31.3.....               | 29.2.....               | 32.0.....               | 28.1.....               | 33.2.....                 |
| CR value (percent).....                                                | 30.3.....               | 21.0.....               | 31.0.....               | 17.5.....               | 33.8.....                 |
| After alkali treatment:                                                |                         |                         |                         |                         |                           |
| Weight decrease ratio (percent).....                                   | 7.2.....                | 15.3.....               | 11.3.....               | 10.8.....               | 6.1.....                  |
| Amount of polyethylene glycol (percent).....                           | 2.3.....                | 5.4.....                | 2.0.....                | 1.6.....                | 1.0.....                  |
| Amount of disodium nonylbenzenephosphonate (percent).....              | 0.....                  | 0.....                  | 2.3.....                | 4.3.....                | 1.0.....                  |
| Water-absorbing property:                                              |                         |                         |                         |                         |                           |
| Before washing.....                                                    | Less than 1 second..... | Less than 1 second..... | Less than 1 second..... | Less than 1 second..... | 2 minutes.....            |
| After 10 washings.....                                                 | 1 second.....           | 1 second.....           | 1 second.....           | do.....                 | More than 10 minutes..... |
| After 50 washings.....                                                 | 5 minutes.....          | 4 minutes.....          | do.....                 | do.....                 | do.....                   |
| Heat resistance (change in <i>b</i> value).....                        | +1.8.....               | +3.8.....               | +2.2.....               | +7.8.....               | +1.7.....                 |

From the results shown in Table 15, the following matters can be seen:

As in the case of Comparative Example 20, the filaments containing polyethylene glycol and having pores therein but being free of disodium nonylbenzenephosphonate are inferior in washing resistance of the water-absorbing property. As in the case of Comparative Example 21, even if the amount of polyethylene glycol is increased in Comparative Example 20, the washing resistance of the water-absorbing property is not improved, and moreover the heat resistance and the CR value of the processed yarn are lowered. As in the case of Comparative Example 22, in case the amount of disodium nonylbenzenephosphonate is too large, the CR value of the processed yarn is low and the heat resistance is degraded. As in the case of Comparative Example 23, even if filaments contain polyethylene glycol and disodium nonylbenzenephosphonate and the weight decrease is observed after the alkali treatment, a sufficient water-absorbing property is not imparted to the filaments when the weight decrease is due only to the surface falling and the polyethylene glycol contained in the form of stripes inside the filaments is not extracted. Thus, it is seen that the results given in Table 15 demonstrate clearly the effects of the present invention.

ments after the elution treatment contained disodium nonylbenzenephosphonate in an amount of 1.0%. Thus, it is seen that the polystyrene portion incompatible with the polyester had been eluted out from the filaments and there were contained fine pores in the filaments. The water-absorbing property of the so treated filaments was characterized by 4 minutes before washing, more than 10 minutes after 10 washings and more than 10 minutes after 50 washings. The water-absorbing property of a knitted product of the filaments prepared without addition of polystyrene by conducting the spinning, drawing, processing and knitting in the same manner as above was characterized by more than 10 minutes before washing. The water-absorbing property of a knitting product obtained by subjecting the above mentioned knitted product to an alkali treatment with a weight decrease ratio of 6.1% was characterized by 4 minutes before washing and more than 10 minutes after 10 washings. In this alkali-treated knitted product the content of disodium nonylbenzenephosphonate was 1.3%, and fine pores were not present in the filaments because disodium nonylbenzenephosphonate was compatible with the polyester.

#### EXAMPLE 17

This example is given to show that even when fine pores are formed by a method different from the method

adopted in Example 15, the effects of the present invention can be fully achieved.

Prior to the initiation of the preparation of polyethylene terephthalate, polyethylene glycol having a molecular weight of 20,000 was added to the polymerization system in an amount of 3.1% by weight, and 2.5% by weight of sodium stearate was added after completion of the polymerization. Thus, there was obtained polymer having an intrinsic viscosity of 0.663. In the same manner as in Comparative Example 24 the polymer was blend-spun with polystyrene, drawn, processed, knitted and treated with trichlene. After the trichlene treatment the amount incorporated of polyethylene glycol was 2.9%, and the amount incorporated of sodium stearate was 1.1%. The polystyrene in an amount of 9.0% was eluted out and fine pores were formed in the filaments.

The water-absorbing property of the product was characterized by 8 seconds after 50 washings.

#### EXAMPLES 18 TO 21 AND COMPARATIVE EXAMPLES 25 TO 26

These examples are given to show what changes are brought about when the class of the polyalkylene ether to

From the results shown in Table 16, the following matters can be seen:

In Comparative Example 25, since the polyethylene glycol was not selectively eluted and fine pores were not formed in the filaments, they do not exhibit a sufficient water-absorbing property. In Comparative Example 26, since the content of the polyalkylene ether in the filaments was too small, the filaments do not exhibit a sufficient water-absorbing property. Thus, it is seen that the results given in Table 16 demonstrate clearly the effects attained by the present invention.

#### EXAMPLES 22 TO 24

These examples are given to show what changes are brought about by varying the class of the metal salt derivative in Example 15.

The experiments were conducted in the same manner as in Example 15 except using other metal salt derivative instead of disodium nonylbenzenephosphonate.

The results are shown in Table 17 below.

TABLE 17

|                                                                 | Example 22                | Example 23              | Example 24                          |
|-----------------------------------------------------------------|---------------------------|-------------------------|-------------------------------------|
| Class of metal salt derivative.....                             | Sodium dodecyl-sulfinate. | Potassium stearate..    | Manganese nonylbenzene phosphonate. |
| Properties of processed yarn:                                   |                           |                         |                                     |
| Strength (g./d.).....                                           | 4.4.....                  | 4.3.....                | 4.2.....                            |
| Elongation (percent).....                                       | 33.2.....                 | 32.6.....               | 33.1.....                           |
| CR value (percent).....                                         | 35.2.....                 | 33.2.....               | 34.6.....                           |
| After alkali treatment:                                         |                           |                         |                                     |
| Weight decrease ratio (percent).....                            | 8.2.....                  | 8.3.....                | 8.2.....                            |
| Amount incorporated of polyethylene glycol (percent).....       | 1.5.....                  | 1.4.....                | 1.5.....                            |
| Amount incorporated of metal salt derivative (percent).....     | 1.0.....                  | 1.2.....                | 1.1.....                            |
| Water absorbing property:                                       |                           |                         |                                     |
| Before washing.....                                             | Less than 1 second.....   | Less than 1 second..... | Less than 1 second.....             |
| After 10 washings.....                                          | do.....                   | do.....                 | Do.....                             |
| After 50 washings.....                                          | 3 seconds.....            | 5 seconds.....          | 4 seconds.....                      |
| Heat resistance after alkali treatment (change in b value)..... | +2.1.....                 | +2.2.....               | +2.4.....                           |

be incorporated is varied in Example 15.

The experiments were conducted in the same manner as in Example 15 except changing the class of the polyalkylene ether to be incorporated. The results are shown in Table 16 below.

#### EXAMPLES 25 TO 26 AND COMPARATIVE EXAMPLES 27 TO 31

Frictional electrification voltages of various knitted products were measured at 20° C. and a relative humidity

TABLE 16

|                                                                        | Example 18                         | Comparative Example 25            | Example 19                        | Example 20                                              | Comparative Example 26            | Example 21                        |
|------------------------------------------------------------------------|------------------------------------|-----------------------------------|-----------------------------------|---------------------------------------------------------|-----------------------------------|-----------------------------------|
| Class of polyalkylene ether.....                                       | Polypropylene glycol. <sup>1</sup> | Polyethylene glycol. <sup>2</sup> | Polyethylene glycol. <sup>1</sup> | Ethylene oxide/pro-pylene oxide copolymer. <sup>3</sup> | Polyethylene glycol. <sup>4</sup> | Polyethylene glycol. <sup>5</sup> |
| Property of processed yarn:                                            |                                    |                                   |                                   |                                                         |                                   |                                   |
| Strength (g./d.).....                                                  | 4.5.....                           | 4.1.....                          | 4.2.....                          | 4.6.....                                                | 4.3.....                          | 4.3.....                          |
| Elongation (percent).....                                              | 31.2.....                          | 27.8.....                         | 30.1.....                         | 33.1.....                                               | 31.0.....                         | 30.3.....                         |
| CR value (percent).....                                                | 30.0.....                          | 22.0.....                         | 26.3.....                         | 30.5.....                                               | 27.9.....                         | 30.2.....                         |
| After alkali treatment:                                                |                                    |                                   |                                   |                                                         |                                   |                                   |
| Weight decrease ratio (percent).....                                   | 7.7.....                           | 7.6.....                          | 8.1.....                          | 7.9.....                                                | 7.9.....                          | 7.8.....                          |
| Amount incorporated of polyalkylene ether (percent).....               | 0.9.....                           | 4.9.....                          | 2.2.....                          | 1.2.....                                                | 0.2.....                          | 1.3.....                          |
| Amount incorporated of disodium nonylbenzenephosphonate (percent)..... | 1.1.....                           | 1.1.....                          | 1.1.....                          | 1.2.....                                                | 1.4.....                          | 1.4.....                          |
| Water absorbing property:                                              |                                    |                                   |                                   |                                                         |                                   |                                   |
| Before washing.....                                                    | Less than 1 second.....            | 3 minutes.....                    | Less than 1 second.....           | Less than 1 second.....                                 | 4 seconds.....                    | Less than 1 second.....           |
| After 10 washings.....                                                 | do.....                            | More than 10 minutes.....         | 1 second.....                     | do.....                                                 | 4 minutes.....                    | Do.....                           |
| After 50 washings.....                                                 | 1 second.....                      | do.....                           | 8 second.....                     | do.....                                                 | More than 10 minutes.....         | 3 seconds.....                    |
| Heat resistance after alkali treatment (change in b value).....        | +2.8.....                          | +2.9.....                         | +2.4.....                         | +2.1.....                                               | +2.0.....                         | +2.0.....                         |

<sup>1</sup> Having a molecular weight of 6,000.

<sup>2</sup> Having a molecular weight of 600.

<sup>3</sup> Having a molecular weight of 21,000 (copolymerization ratio=1:1).

<sup>4</sup> Both terminal ends of which are blocked with  $-\text{OCH}_3$  (molecular weight=16,000).

<sup>5</sup> One terminal end of which is blocked with phosphoric acid (molecular weight=10,000);

of 43% by means of a rotary static tester. The results are shown in Table 18 below.

TABLE 18

| Sample                 | Frictional electrification voltage (v.)                                                                                    |        |
|------------------------|----------------------------------------------------------------------------------------------------------------------------|--------|
| Example 25             | Knitted product of Example 15                                                                                              | 2,000  |
| Comparative Example 27 | Knitted product of the control described in Example 15                                                                     | 10,000 |
| Comparative Example 28 | Knitted product of Comparative Example 20                                                                                  | 6,800  |
| Comparative Example 29 | Knitted product of Comparative Example 21                                                                                  | 7,000  |
| Example 26             | Knitted product of Example 16                                                                                              | 2,200  |
| Comparative Example 30 | Knitted product of Comparative Example 23                                                                                  | 8,500  |
| Comparative Example 31 | Knitted product obtained by conducting the eluting treatment after the incorporation of polystyrene in Comparative Ex. 24. | 7,200  |

It is seen that the results given in Table 18 clearly demonstrate the effects attained by the present invention.

#### EXAMPLE 27 AND COMPARATIVE EXAMPLES 32 TO 34

These examples are given to show the correspondence of the water-absorbing time used as the criterion for evaluation of the water-absorbing property to the stuffy uncomfortable feeling of wearers.

With respect to each of a knit underwear of the product of Example 15, a knit underwear of the control products described in Example 15, a knit underwear of the product of Comparative Example 20, and a commercially available knit underwear of pure cotton having a weight of  $17 \times 10^{-3}$  g./cm.<sup>2</sup>, 10 men having an age of 20 to 25 years put on such knit underwear and were allowed to stay for 3 hours at a room maintained constantly at 27° C. and a relative humidity of 65%, and the number of men complaining of a stuffy uncomfortable feeling was recorded. The tests were conducted with respect to either the underwears before washing or the underwears after 50 washings. The results are shown in Table 19.

15 speed of 400 m./min. by means of a hot pin heated at 100° C.

The resulting drawn filaments were characterized by a fineness of 74.7 d., a strength of 4.9 g./d., an elongation of 28.1% and a boiling water shrinkage of 13.1%. Two 20 of the drawn filaments were gathered and then subjected to a wooly-processing treatment at a yarn feed rate of 49.8 m./min., a take-up rate of 4.40 m./min. and a hot plate temperature of 205° C. with the use of a spindle rotating at 175,000 r.p.m. The so obtained wooly-processed 25 yarn were characterized by a strength of 4.4 g./d., an elongation of 30.3%, and a CR value (crimp retaining property) of 34.8%. A knitted cloth having a weight of  $15-18 \times 10^{-3}$  g./cm.<sup>2</sup> was prepared from the above 30 wooly-processed yarn, and it was scoured at 80° C. for 20 minutes under the conditions of a cleanser of 2 g./liter, soda ash of 1 g./liter and a bath ratio of 1:100. Then, the scoured cloth was treated for 20 minutes with a 35 0.3 N aqueous solution of sodium hydroxide at the boiling point of the solution.

TABLE 19

| Sample                 | Number of men complaining of stuffy uncomfortable feeling |                   |   |
|------------------------|-----------------------------------------------------------|-------------------|---|
|                        | Before washing                                            | After 50 washings |   |
| Example 27             | Underwear of the product of Example 15                    | 1                 | 1 |
| Comparative Example 32 | Underwear of the control described in Example 15          | 9                 | 9 |
| Comparative Example 33 | Underwear of the product of Comparative Example 20        | 3                 | 8 |
| Comparative Example 34 | Underwear of pure cotton                                  | 1                 | 1 |

#### EXAMPLE 28 AND COMPARATIVE EXAMPLE 35

Polyethylene terephthalate (A) of an intrinsic viscosity of 0.660 containing 0.5% of titanium oxide as a delustering agent and obtained by a customary method

Before and after the said alkali treatment, the weight decrease ratio, the amount of polyethylene glycol and the amount of disodium nonylphenolphosphoric acid ester were measured. The results are shown in Table 20 below.

TABLE 20

|                                                  | Weight decrease ratio, percent | Amount of polyethylene glycol, percent | Amount of disodium nonylphenolphosphoric acid ester, percent |
|--------------------------------------------------|--------------------------------|----------------------------------------|--------------------------------------------------------------|
| Comparative Example 35 (before alkali treatment) | 0                              | 4.9                                    | 2.5                                                          |
| Example 28 (after alkali treatment)              | 8.3                            | 1.7                                    | 1.0                                                          |

was weighed at 295° C. by means of a gear pump, and then fed to a kneading screw portion heated at 285° C. A 2:1 mixture (B) of polyethylene glycol having a number average molecular weight of 20,000 and disodium nonylphenolphosphoric acid ester was weighed at 85° C. by means of a gear pump, and then fed to the kneading screw portion heated at 285° C.

The mixing ratio of (A) and (B) was 92.5:7.5. The mixture was transferred from the kneading screw portion to a spinneret portion while being kept in the molten state. Then, the molten mixture was spun at a rate of 30 g./min. through a spinneret having 36 nozzles of a 0.23 mm. diameter. The extrudate was taken up at a rate

65 of the drawn yarn after the scouring and alkali treatments were shown in FIGS. 9 and 10. FIG. 11 is an electromicroscopic photo of FIG. 9, after it has been dyed with osmium tetroxide and dissolved. FIG. 12 is an electromicroscopic photo of the yarn of FIG. 10, after 70 it has been dyed with osmium tetroxide and dissolved.

From the results given in Table 20, and FIGS. 9 to 12, it is seen that in the yarn before the alkali treatment the polyethylene glycol was incorporated in the form of stripes and that a part of the polyethylene glycol corresponding to 3.2% of the total yarn was stripped off by the

## 23

alkali treatment to form fine pores. It is also seen that in addition to the polyethylene glycol and disodium nonylphenolphosphoric acid ester, the polyethylene terephthalate per se was stripped off in an amount of 3.6% by the alkali treatment, and hence, the yarn was made thinner and the pores were expanded from their interior. From FIG. 12, it is observed that the diameter of the pore was about  $0.1\mu$  and the length-to-diameter ratio was greater than 10.

With respect to the knitted cloth of the yarn before the alkali treatment and the knitted cloth of the yarn after the alkali treatment, the water-absorbing property was measured. The results are shown in Table 21 below.

TABLE 21

|                                                       | Before washing          | After 10 washings       | After 50 washings       |
|-------------------------------------------------------|-------------------------|-------------------------|-------------------------|
| Comparative Example 35 (before alkali treatment)..... | More than 10 minutes.   | More than 10 minutes.   | More than 10 minutes.   |
| Example 28 (after alkali treatment).....              | Less than 1 second..... | Less than 1 second..... | Less than 1 second..... |

From the results shown in Table 21 it is seen that even 20 or polyethylene glycol and disodium nonylphenolphosphoric acid ester incorporated in the polyester. The results are shown in Table 24 below.

TABLE 24

|                                                                                 | Comparative Example 36  | Comparative Example 37  | Example 29              | Comparative Example 38  | Comparative Example 39    |
|---------------------------------------------------------------------------------|-------------------------|-------------------------|-------------------------|-------------------------|---------------------------|
| Amount incorporated of polyethylene glycol (percent).....                       | 5.0.....                | 15.0.....               | 5.0.....                | 5.0.....                | 1.0.....                  |
| Amount incorporated of disodium nonylphenolphosphoric acid ester (percent)..... | 0.....                  | 0.....                  | 5.0.....                | 10.0.....               | 1.0.....                  |
| Properties of processed yarn:                                                   |                         |                         |                         |                         |                           |
| Strength (g./d.).....                                                           | 4.6.....                | 3.7.....                | 4.3.....                | 3.5.....                | 4.6.....                  |
| Elongation (percent).....                                                       | 31.0.....               | 27.2.....               | 30.0.....               | 27.0.....               | 31.5.....                 |
| CR value (percent).....                                                         | 34.0.....               | 21.0.....               | 30.3.....               | 17.1.....               | 34.2.....                 |
| After alkali treatment:                                                         |                         |                         |                         |                         |                           |
| Weight decrease ratio (percent).....                                            | 7.2.....                | 10.1.....               | 10.5.....               | 10.2.....               | 6.0.....                  |
| Amount of polyethylene glycol (percent).....                                    | 2.0.....                | 5.8.....                | 1.8.....                | 1.6.....                | 1.0.....                  |
| Amount of disodium nonylphenolphosphoric acid ester (percent).....              | 0.....                  | 0.....                  | 2.2.....                | 4.3.....                | 1.0.....                  |
| Water absorbing property:                                                       |                         |                         |                         |                         |                           |
| Before washing.....                                                             | Less than 1 second..... | Less than 1 second..... | Less than 1 second..... | Less than 1 second..... | 2 minutes.....            |
| After 10 washings.....                                                          | 1 second.....           | 1 second.....           | do.....                 | do.....                 | More than 10 minutes..... |
| After 50 washings.....                                                          | 4 minutes.....          | 4 minutes.....          | do.....                 | do.....                 | Do.....                   |
| Heat resistance after alkali treatment (change in <i>b</i> value).....          | +1.8.....               | +3.0.....               | +2.2.....               | +8.1.....               | +1.8.....                 |

absorbing property unless they have fine pores therein.

Table 22 shows the results of the measurement of the heat resistance of the knitted clothes of the yarn before the alkali treatment and of the yarn after the alkali treatment.

TABLE 22

| Example No:                                           | Heat resistance<br>(change in <i>b</i> value) |
|-------------------------------------------------------|-----------------------------------------------|
| Comparative Example 35 (before alkali treatment)..... | +2.1.....                                     |
| Example 28 (after alkali treatment).....              | +1.9.....                                     |

For comparison sake, properties of ordinary polyester filaments (control) prepared without addition of polyethylene glycol and disodium nonylphenolphosphoric acid ester were examined. The spinning, drawing, wooly-processing, knitting and alkali treatment were conducted in the same manner as described above. The drawn yarn was characterized by a fineness of 74.9 d., a strength of 4.7 g./d., an elongation of 27.5% and a boiling water shrinkage of 12.0%. The wooly-processed yarn was characterized by a strength of 4.5 g./d., an elongation of 33.5% and a CR value of 37.2%. The weight decrease ratio by the alkali treatment was 2.2%. The water-absorbing property of the knitted cloth was as follows.

From the results shown in Table 24, the following matters can be seen:

As in the case of Comparative Example 36, the filaments containing polyethylene glycol and having pores therein but being free of disodium nonylphenolphosphoric acid ester are inferior in washing resistance of the water-absorbing property. As in the case of Comparative Example 37, even if the amount of polyethylene glycol was increased in Comparative Example 36, the washing resistance of the water-absorbing property is not improved, and moreover the heat resistance and the CR value of the processed yarn are lowered. As in the case of Comparative Example 38, in case the amount of disodium nonylphenolphosphoric acid ester is too large, the CR value of the processed yarn is low and the heat resistance is degraded. As in the case of Comparative Example 39, even if filaments contain polyethylene glycol and disodium nonylphenolphosphoric acid ester and the weight decrease is observed after the alkali treatment, a sufficient water-absorbing property is not given to the filaments when the weight decrease is due only to the surface falling and the polyethylene glycol contained in the form of stripes inside the filaments is not extracted. Thus, it is seen that the results given in Table 24 demonstrate clearly the effects of the present invention.

TABLE 23

|                              | Before washing            | After 10 washings         | After 50 washings         |
|------------------------------|---------------------------|---------------------------|---------------------------|
| Before alkali treatment..... | More than 10 minutes..... | More than 10 minutes..... | More than 10 minutes..... |
| After alkali treatment.....  | 5 minutes.....            | do.....                   | Do.....                   |

The heat resistance expressed in terms of the change in *b* value of the knitted cloth was +1.5 either before or after the alkali treatment.

## 24

EXAMPLE 29 AND COMPARATIVE EXAMPLES  
36 TO 39

These examples were given to show what phenomena are brought about by changing the amounts incorporated of polyethylene glycol and disodium nonylphenolphosphoric acid ester in the polyester of Example 28.

The experiments were conducted in the same manner as in Example 28 except changing the mixing ratio of polyethylene glycol and disodium nonylphenolphosphoric acid ester, the incorporation ratio of the mixture of polyethylene glycol and disodium nonylphenolphosphoric acid ester to polyethylene terephthalate or the amounts

## COMPARATIVE EXAMPLE 40

This example is given to show that a sufficient water-absorbing property is not imparted to filaments contain-

ing only disodium nonylphenylphosphoric acid ester, filaments obtained by subjecting the above filaments to an alkali treatment, and filaments containing disodium nonylphenylphosphoric acid ester and having fine pores therein.

To polyethylene terephthalate of Example 28, 2.5% of disodium nonylphenylphosphoric acid ester was added after completion of the polymerization. Thus, there was obtained a polymer having an intrinsic viscosity of 0.658.

The so obtained polymer (A) was weighed at 295° C. by means of a gear pump and fed to a kneading screw portion heated at 285° C. Polystyrene (B) ("Styron 666," product of Asahi Dow Chemical Industry Co.) was weighed at 180° C. by means of a gear pump and fed to the kneading screw portion heated at 285° C. The mixing ratio of (A) to (B) was 90:10.

Thereafter, the spinning, drawing, processing and knitting were conducted in the same manner as in Example 28, and then the polystyrene was eluted with trichlene at its boiling point. The weight decrease ratio was 9.0% at this elution treatment. It was confirmed that the filaments after the elution treatment contained disodium nonylphenylphosphoric acid ester in an amount of 1.1%. Thus it is seen that the polystyrene portion incompatible with the polyester had been eluted out from the filaments, and there were formed fine pores in the filaments. The water-absorbing property of the so treated filaments was characterized by 3 minutes before washing, more than

Prior to the initiation of the preparation of polyethylene terephthalate, polyethylene glycol having a molecular weight of 20,000 was added to the polymerization system in an amount of 3.1% by weight, and 2.5% by weight of monopotassium di(dodecylalcohol)phosphorous acid ester was added after completion of the polymerization. Thus, there was obtained a polymer having an intrinsic viscosity of 0.663. In the same manner as in Comparative Example 40 the polymer was blend-spun with polystyrene, drawn, processed, knitted and treated with trichlene. After the trichlene treatment the amount incorporated of polyethylene glycol was 3.1% and the amount incorporated of monopotassium di(dodecylalcohol)phosphorous acid ester was 1.1%. The polystyrene in an amount of 9.1% was eluted out and fine pores were formed in the filaments.

The water-absorbing property of the product was characterized by 9 seconds after 50 washings.

#### EXAMPLES 31 TO 34 AND COMPARATIVE EXAMPLES 41 TO 42

These examples are given to show what changes are brought about when the class of the polyalkylene ether to be incorporated is varied in Example 28.

The experiments were conducted in the same manner as in Example 28 except changing the class of the polyalkylene ether to be incorporated. The results are shown in Table 25 below.

TABLE 25

|                                                                             | Example 31                         | Comparative Example 41            | Example 32                        | Example 33                                           | Comparative Example 42            | Example 34                        |
|-----------------------------------------------------------------------------|------------------------------------|-----------------------------------|-----------------------------------|------------------------------------------------------|-----------------------------------|-----------------------------------|
| Class of polyalkylene ether                                                 | Polypropylene glycol. <sup>1</sup> | Polyethylene glycol. <sup>2</sup> | Polyethylene glycol. <sup>1</sup> | Ethylene oxide/propane oxide copolymer. <sup>3</sup> | Polyethylene glycol. <sup>4</sup> | Polyethylene glycol. <sup>5</sup> |
| Properties of processed yarn:                                               |                                    |                                   |                                   |                                                      |                                   |                                   |
| Strength (g./d.)                                                            | 4.4                                | 4.0                               | 4.3                               | 4.6                                                  | 4.5                               | 4.4                               |
| Elongation (percent)                                                        | 32.0                               | 27.0                              | 28.2                              | 32.3                                                 | 33.1                              | 28.2                              |
| CR value (percent)                                                          | 31.0                               | 23.0                              | 27.8                              | 32.3                                                 | 29.3                              | 31.2                              |
| After alkali treatment:                                                     |                                    |                                   |                                   |                                                      |                                   |                                   |
| Weight decrease ratio (percent)                                             | 7.6                                | 7.5                               | 8.0                               | 7.8                                                  | 7.9                               | 7.8                               |
| Amount incorporated of polyalkylene ether (percent)                         | 1.0                                | 4.9                               | 2.3                               | 1.3                                                  | 0.2                               | 1.3                               |
| Amount incorporated of disodium nonylphenylphosphorous acid ester (percent) | 1.0                                | 1.2                               | 1.1                               | 1.1                                                  | 1.3                               | 1.3                               |
| Water absorbing property:                                                   |                                    |                                   |                                   |                                                      |                                   |                                   |
| Before washing                                                              | Less than 1 second                 | 3 minutes                         | Less than 1 second                | Less than 1 second                                   | 5 seconds                         | Less than 1 second                |
| After 10 washings                                                           | do                                 | More than 10 minutes              | do                                | do                                                   | 5 minutes                         | do                                |
| After 50 washings                                                           | 1 second                           | do                                | 9 seconds                         | do                                                   | More than 10 minutes              | 3 seconds                         |
| Heat resistance after alkali treatment (change in b value)                  | +2.7                               | +2.8                              | +2.5                              | +2.2                                                 | +2.1                              | +2.0                              |

<sup>1</sup> Having a molecular weight of 6,000.

<sup>2</sup> Having a molecular weight of 600.

<sup>3</sup> Having a molecular weight of 21,000 (copolymerization ratio=1:1).

<sup>4</sup> Both terminal ends of which are blocked with  $-\text{OCH}_3$  (molecular weight=16,000).

One terminal end of which is blocked with phosphoric acid (molecular weight=10,000).

10 minutes after 10 washings and more than 10 minutes after 50 washings. The water-absorbing property of a knitted product of the filaments prepared without addition of polystyrene by conducting the spinning, drawing, processing and knitting in the same manner as above was characterized by more than 10 minutes before washing. The water-absorbing property of a knitted product obtained by subjecting the above mentioned knitted product to an alkali treatment with a weight decrease ratio of 6.2% was characterized by 4 minutes before washing and more than 10 times after 10 washings. In this alkali-treated knitted product the content of disodium nonylphenylphosphoric acid ester was 1.5%, and fine pores were not present in the filaments because disodium nonylphenylphosphoric acid ester was compatible with the polyester.

#### EXAMPLE 30

This example is given to show that even when fine pores are formed by a method different from the method adopted in Example 28, the effects of the present invention can be fully achieved.

From the results shown in Table 25, the following matters can be seen. In Comparative Example 41, since the polyethylene glycol was not selectively eluted and fine pores were not formed in the filaments, they do not exhibit sufficient water-absorbing property. In Comparative Example 42, since the content of the polyalkylene ether is small, the filaments do not exhibit a sufficient water-absorbing property. Thus, it is seen that the results shown in Table 25 demonstrate clearly the effects attained by the present invention.

#### EXAMPLES 35 TO 37

These examples are given to show what changes are brought about by varying the class of the metal salt derivative of phosphoric or phosphorous acid in Example 28.

The experiments were conducted in the same manner as in Example 28 except using other metal salt derivative

instead of disodium nonylphenylphosphoric acid ester. The results are shown in Table 26 below.

TABLE 26

|                                                                   | Example 35                                   | Example 36                                  | Example 37                                     |
|-------------------------------------------------------------------|----------------------------------------------|---------------------------------------------|------------------------------------------------|
| Class of metal salt derivative                                    | Monosodium nonylphenylphosphoric acid ester. | Manganese nonylphenylphosphoric acid ester. | Disodium dodecylalcohol-phosphoric acid ester. |
| Properties of processed yarn:                                     |                                              |                                             |                                                |
| Strength (g./d.)                                                  | 4.5                                          | 4.5                                         | 4.5                                            |
| Elongation (percent)                                              | 32.6                                         | 33.2                                        | 31.6                                           |
| CR value (percent)                                                | 35.2                                         | 36.1                                        | 34.2                                           |
| After alkali treatment:                                           |                                              |                                             |                                                |
| Weight decrease ratio (percent)                                   | 8.2                                          | 8.3                                         | 8.3                                            |
| Amount incorporated of polyethylene glycol (percent)              | 1.4                                          | 1.4                                         | 1.3                                            |
| Amount incorporated of metal salt derivative (percent)            | 1.1                                          | 1.1                                         | 1.2                                            |
| Water absorbing property:                                         |                                              |                                             |                                                |
| Before washing                                                    | Less than 1 second                           | Less than 1 second                          | Less than 1 second                             |
| After 10 washings                                                 | do                                           | do                                          | do                                             |
| After 50 washings                                                 | 1 second                                     | 1 second                                    | 5 seconds                                      |
| Heat resistance after alkali treatment (change in $\delta$ value) | +2.2                                         | +2.3                                        | +2.1                                           |

### EXAMPLES 38 TO 39 AND COMPARATIVE EXAMPLES 43 TO 47

Frictional electrification voltages of various knitted products were measured at 20° C. and a relative humidity of 43% by a rotary static tester. The results are shown in Table 27 below.

TABLE 27

| Sample                 | Frictional electrification voltage (v.)                                                                                    |
|------------------------|----------------------------------------------------------------------------------------------------------------------------|
| Example 38             | Knitted product of Example 28                                                                                              |
| Comparative Example 43 | Knitted product of the control described in Example 28                                                                     |
| Comparative Example 44 | Knitted product of Comparative Example 36                                                                                  |
| Comparative Example 45 | Knitted product of Comparative Example 37                                                                                  |
| Example 39             | Knitted product of Example 29                                                                                              |
| Comparative Example 46 | Knitted product of Comparative Example 39                                                                                  |
| Comparative Example 47 | Knitted product obtained by conducting the eluting treatment after the incorporation of polystyrene in Comparative Ex. 40. |

It is seen that the results given in Table 27 clearly demonstrate the effects attained by the present invention.

### EXAMPLE 40 AND COMPARATIVE EXAMPLES 48 TO 50

These examples are given to show the correspondence of the water-absorbing time used as the criterion for evaluation of the water-absorbing property to the stuffy uncomfortable feeling of wearers.

With respect to each of a knit underwear of the product of Example 28, a knit underwear of the control product described in Example 28, a knit underwear of the product of Comparative Example 36, and a commercially available knit underwear of pure cotton having a weight of  $17 \times 10^{-3}$  g./cm.<sup>2</sup>, 10 men having an age of 20 to 25 years put on such knit underwear and were allowed to stay at a room maintained constantly at 27° C. and a relative humidity of 65%, and the number of men complaining of a stuffy uncomfortable feeling was recorded. The tests were conducted with respect to either the underwears before washing or after 50 washings. The results are shown in Table 28.

TABLE 28

| Sample                 | Number of men complaining of stuffy uncomfortable feeling |                   |
|------------------------|-----------------------------------------------------------|-------------------|
|                        | Before washing                                            | After 50 washings |
| Example 40             | Underwear of the product of Example 28                    | 1                 |
| Comparative Example 48 | Underwear of the control product described in Example 28  | 9                 |
| Comparative Example 49 | Underwear of the product of Comparative Example 36        | 2                 |
| Comparative Example 50 | Underwear of pure cotton                                  | 1                 |
|                        |                                                           | 1                 |
|                        |                                                           | 8                 |

### EXAMPLE 41

Each of a knitted product obtained in Example 1, an alkali-treated knitted product of ordinary polyethylene terephthalate processed yarn described as control in Example 1 and a commercially available knitted product described in Comparative Example 18 was washed 20 times. Then water-absorbing properties of these products were examined by employing the apparatus shown in FIG. 13.

group consisting of metal salt derivatives of carboxylic acid, phosphonic acid and sulfinic acid.

4. Polyester filaments of claim 1 wherein said metal salt derivative is at least one member selected from the group consisting of di-metal salts and mono-metal salts of phosphoric acid and phosphorous acid.

5. The polyester filaments of claim 1 wherein said polyalkylene ether is present in an amount of from 1-4% by weight.

The results are shown in FIG. 14. In FIG. 14, curves *a*, *b* and *c* show measurement results of the product of

6. The polyester filaments of claim 1 wherein said metal salt derivative is present in an amount of from 0.3-2.5% by weight.

7. The polyester filaments of claim 2 wherein said alkali metal sulfonate derivative has one sulfonic group and a hydrophobic group in addition thereto.

8. The polyester filaments of claim 3 wherein said metal salt derivative has at least one hydrophilic group and hydrophobic group.

9. The polyester filaments of claim 4 wherein the remaining hydroxy groups of said di-metal salts and mono-metal salts of phosphoric acid and phosphorus acid are in the form of alkylaryl esters. 10

## References Cited

## UNITED STATES PATENTS

5 3,329,557 7/1967 Magat et al. \_\_\_\_\_ 260—857

SAMUEL H. BLECH, Primary Examiner

M. FOELAK, Assistant Examiner

U.S. Cl. X.R.

260—2.5 M, 2.5 E, 860, 873; 264—49, 210 F, 290 T